

W. H. WINSLOW.  
PROCESS OF MAKING BOILERS.  
APPLICATION FILED MAR. 8, 1912.

1,281,247.

Patented Oct. 8, 1918.



Witnesses:  
Albert G. McCabe.  
Robert F. Brache

By

Inventor  
William H. Winslow  
Howard Williams  
Attorneys

# UNITED STATES PATENT OFFICE.

WILLIAM H. WINSLOW, OF CHICAGO, ILLINOIS, ASSIGNOR TO WINSLOW SAFETY HIGH-PRESSURE BOILER CO., A CORPORATION OF ILLINOIS.

## PROCESS OF MAKING BOILERS.

1,281,247.

Specification of Letters Patent.

Patented Oct. 8, 1918.

Application filed March 8, 1912. Serial No. 682,483.

*To all whom it may concern:*

Be it known that I, WILLIAM H. WINSLOW, a citizen of the United States, residing at Chicago, in the county of Cook and State 5 of Illinois, have invented a certain new and useful Improvement in Processes of Making Boilers, of which the following is a full, clear, concise, and exact description, reference being had to the accompanying drawings, forming a part of this specification.

My invention relates to an improved process for making boilers by which the various parts of the boiler structure are secured together so as to make them a single unitary 15 structure, and in addition so treating the parts thus secured together that all internal strains are relieved.

More specifically, my invention consists in taking the various parts of a steel boiler 20 and securing them together by means of the oxy-acetylene blowpipe, so that the adjoining portions of the various parts flow together, thus uniting the parts into a single homogeneous structure, in which the metal 25 is continuous through the structure, after which the completed structure is heated sufficiently, preferably to redness, so that the molecules of the structure may readily assume positions entirely relieving any internal 30 strains that may have existed after the fusing operation and manufacturing of the tubes. The structure thus heated is carefully cooled so that there is no chance of introducing unequal strains in the structure 35 by the cooling operation.

As is well known in the art, standard steel tubing such as is generally available for making boiler structures of different kinds is somewhat tempered or hardened, as a result 40 of its manufacture, and, furthermore, the hardness is apt to be somewhat different at different points in the tubes. By my process the joints between adjoining parts of a boiler structure in which such tubes are employed 45 are made comparatively soft by the fusing of the parts together, and I find it is advisable in order to entirely eliminate internal strains to anneal the entire structure after it is made, so that the tubes may be given 50 a uniform condition as to hardness throughout, and, furthermore, that the entire structure may have a substantially uniform condition of hardness so that the sub-

sequent application of heat to it will not produce unequal strains tending to break down or warp the structure.

My invention is not limited to the construction of boilers of any particular type, but may be employed equally well with either fire-tube or water-tube boilers, and it 60 may also be applied either to boilers of the so-called "flash" type or to those in which a water level is employed.

The several drawings illustrating my invention are as follows:

Figure 1 shows a boiler in which water tubes are employed.

Fig. 2 shows a boiler in which fire tubes are employed, the boiler being of the water-level type.

Fig. 3 shows a boiler in which a water tube is employed, the boiler being of the flash type.

Similar numerals refer to similar parts throughout the several views.

As shown in Fig. 1, the water tubes 1 extend between two vertical headers 2 and 3, the ends of the tubes 1 being secured to the headers 2 and 3 by fusion by means of the oxy-acetylene blowpipe, so that the joints 80 result in a continuous metal structure from one part to another, as indicated at 4. A water header 5 is employed to supply water to the boiler and a steam header 6 serves to collect and remove from the boiler the steam 85 generated.

In the structure shown in Fig. 2, the tubes 7 are secured in the boiler heads 8 and 9 by fusion by means of the oxy-acetylene flame, so that the metal is continuous from the 90 tubes to the heads, and the head 8 is secured into the shell 10 by the same means. In Fig. 2, the boiler shown has its head 9 formed integrally with the shell 10, so that no operation is necessary for securing these parts 95 together.

In the modified construction shown in Fig. 3, the flash coils 11 and 12 are secured together, as indicated at 13, by fusion by means of the oxy-acetylene flame, and the ends of 100 the coils are also secured to the water header 14 and the steam header 15 in a similar way, as a result of which a single homogeneous structure results.

The particular boiler constructions shown 105 in Figs. 1, 2 and 3 do not constitute a part

of the present invention but are shown herein to indicate the adaptability of my process of making boilers to boilers of various types.

While my invention consists broadly in 5 making a boiler structure by fusing the parts together so that they constitute a single homogeneous structure and then heating the resulting structure sufficiently so that unequal internal strains are eliminated, it will 10 be understood that my invention is particularly applicable to steel boiler structures, since parts made of steel are more apt to have internal strains resulting from their construction than are parts made of softer 15 metal. By the term "steel" as used in this connection, I mean to include all forms of steel or iron, whether used in combination with other substances or not, which may be used in forming boiler structures of any type 20 desired.

What I claim is:

1. The process of forming a boiler which consists in placing edge to edge a plurality of thin-walled steel parts forming part of a 25 closed vessel, then fusing the adjacent edges only and flowing the fused metal at said edges together to unite the adjacent edges, then heating the structure resulting from the parts so joined, to substantially a red 30 heat and then slowly cooling to relieve the internal stresses in the metal.

2. The process of forming a plurality of tubes of different lengths and diameters into boiler sections, which consists in placing 35 the tubes at the points where joints are to be made, with their edges together, then heating adjacent edges only to the point of fusion and flowing the metal of the edges together, then allowing the fused metal to cool 40 to a point where the entire structure is self-supporting, then heating the entire structure to substantially red heat to relieve internal stresses, and then slowly cooling.

3. The process of making boilers which

consists in fusing together the parts of the 45 structure to form a hollow containing structure by melting the adjoining edges of the parts and flowing them together, and annealing the resulting structure by heating the same sufficiently to relieve the structure of 50 its internal strains.

4. The process of making a boiler consisting of fusing the parts of metal tubes to suitable coöperating parts to form a substantially closed steam container by melting 55 the adjoining parts until they flow together, heating the resulting structure sufficiently to equalize its internal strains, and slowly cooling the heated structure.

5. The process of treating a steel boiler 60 constructed of parts of different lengths or thickness united by molecular union of said parts, which consists in heating said entire boiler to substantially red heat and thereafter slowly cooling the same.

6. The process of forming and treating a steel boiler which process consists in joining together constituent parts of a boiler to form a hollow substantially closed structure, then heating said entire boiler structure to substantially red heat and thereafter slowly cooling the same.

7. The process of constructing a boiler which process consists in welding together a plurality of tubes of different lengths to 75 and between a pair of risers communicating with all of said tubes to form a substantially closed boiler structure, and then heating said entire boiler structure to a red heat and then slowly cooling same.

In witness whereof, I hereunto subscribe my name this 29th day of February, A. D. 1912.

WILLIAM H. WINSLOW.

Witnesses.

ALBERT C. BELL,  
ALBIN C. AHLBERG.